

1

3,288,713  
SYNTHETIC ESTER LUBRICANTS CONTAINING  
ANTIOXIDANTS

Daniel B. Eickemeyer, Park Forest, and Tai S. Chao,  
Homewood, Ill., assignors to Sinclair Research, Inc.,  
New York, N.Y., a corporation of Delaware  
No Drawing. Filed Nov. 14, 1963, Ser. No. 323,562  
11 Claims. (Cl. 252—51.5)

This invention relates to ester-based lubricant compositions containing a novel combination of base oil-soluble additive agents. More particularly, the present invention relates to ester-based synthetic lubricant compositions which exhibit increased oxidation resistance.

Organic compounds, such as lubricating oils, undergo oxidation upon exposure to air. This process is accentuated by elevated temperatures such as occur in engines and other operating machinery. When such organic compositions are used as motor or machinery lubricants, their stability is still further drastically reduced due to their contact with metal surfaces which give up metallic particles to the lubricant. Such abraded or dissolved metals or metal salts appear to act as oxidation catalysts in the lubricant causing the formation of primary oxidation products which in turn cause further degradation of the organic compounds present in the composition. In addition, water also causes corrosion of metallic surfaces and accentuates oxidation of the lubricant.

Problems of this nature are encountered in mineral oils but appear to be particularly troublesome in synthetic oleaginous fluids exemplified by esters. Ordinarily, these synthetic ester fluids can be effectively inhibited against oxidation by the use of small amounts of additives. However, in the presence of certain metals and metal compounds often occurring in the lubricants, particularly as aforementioned, through contact with metal surfaces such as iron, the effectiveness of the additives is greatly reduced.

The present invention provides a synthetic ester-based lubricant containing a primary antioxidant and certain N-substituted amino compounds. The N-substituted amino compounds of the invention can be represented by the following general formula:



wherein X is a pyridyl or quinolyl radical and can be substituted as with straight or branched chain alkyl groups of 1 to 12 carbon atoms, preferably 1 to 8 carbon atoms, or with other non-interfering substituents such as hydroxy or alkoxy groups; and R is an n-valent hydrocarbon radical of up to 16 or even, 20, 24 or more carbon atoms whose adjacent carbon atoms are no closer than 1.40 Å., (i.e., a non-olefinic, non-acetylenic hydrocarbon. Thus R may be an aromatic hydrocarbon radical-containing n-valent hydrocarbon radical. R can be an aryl or mixed aryl-alkyl radical. R can also be substituted with non-interfering groups such as hydroxyl, alkyl and alkoxy groups. R is often phenyl, including substituted phenyl, phenyl-substituted lower alkyl or a mixed phenyl-lower alkyl radical. The integer n is a value of 1 to 2.

Examples of preferred groups of N-substituted amino compounds contemplated by the present invention are:

A. N-substituted aminopyridine represented by the structural formula:



wherein R<sub>1</sub> is hydrogen or an alkyl group of 1 to 12 carbon atoms, preferably 1 to 8 carbon atoms, and R<sub>2</sub>

2

is a hydrocarbyl, aryl or alkyl group of 1 to 12 carbon atoms;

B. N-substituted aminoquinoline having the structural formula:



wherein R<sub>1</sub> and R<sub>2</sub> are as defined in A above and R<sub>1</sub> and NHR<sub>2</sub> are on different carbon atoms of positions 2 to 8.

C. The condensation product of aldehyde and aminopyridines having the structural formula:



wherein R<sub>1</sub> is as identified in A above and R<sub>3</sub> is an alkyl group of 1 to 12, preferably 1 to 8 carbon atoms. Any process known in the art for the production of these products can be employed as, for example, heating to reaction temperature, usually about 70 to 150° C., at least 2 moles of the aminopyridine with 1 mole of an aldehyde of 1 to 12 carbon atoms, preferably in the presence of an azeotroping solvent such as toluene.

D. The condensation product of aminopyridine, aldehyde and alkylphenol having the structural formula:



wherein R<sub>1</sub> is as defined in A above; R<sub>4</sub> is a divalent alkyl radical of 1 to 4 carbon atoms and R<sub>5</sub> is an alkyl group of 1 to 8 carbon atoms, preferably a tertiary alkyl radical located in a position para to the hydroxy substituents, for instance as in



These compounds like those of C above can be prepared by known condensation methods, for instance, by reacting together 2 moles of an aminopyridine, 2 moles of an aldehyde of 1 to 4 carbon atoms and 1 mole of an alkylphenol in the presence of an azeotroping solvent for water.

The primary antioxidant component of the invention is an aromatic amine which is soluble in the ester fluid to extent used and can be represented by the following general formula:



wherein Q is a monovalent hydrocarbon of 1 to 20 carbons, preferably 6 to 12 carbon atoms, whose adjacent carbon atoms are no closer than 1.40 Å., (i.e., a non-olefinic, non-acetylenic, monovalent hydrocarbon), and Q' is an aromatic hydrocarbon radical of 6 to 12 or 16 carbon atoms. Thus Q can be an alkyl group, including cycloalkyl, or an aromatic group. Preferably, both Q and Q' are aromatic and often at least one is a fused ring aromatic, e.g., naphthyl. Q and Q' can be substituted with non-interfering substituents such as alkyl groups

and amine groups, preferably alkyl or aromatic amines, and Q and Q' can be linked together by means of a non-interfering element such as carbon, sulfur and oxygen.

Illustrative of suitable amines are phenothiazine, N-phenyl- $\alpha$ -naphthyl amine; di( $\alpha$ -naphthyl amine); N,N-diphenyl paraphenylene diamine; N,N-diethyl para-phenylene diamine, N,N-heptylphenyl-para-phenylene diamine; diphenyl amine, N-butyl phenyl-( $\alpha$ -decyl) amine, etc.

The additives of the present invention are used in minor amounts sufficient to retard oxidation of the synthetic lubricant at temperatures in excess of 400° F. The actual amount of the additives employed may depend upon the particular lubricant utilized and the particular N-substituted amino compound selected. Ordinarily about 0.1 to 5% by weight, more often about .1 to 1.5% by weight, of each inhibitor based on the final composition is employed.

The lubricant composition of this invention includes as the major component a base oil which is an ester of lubricating viscosity which may be, for instance, a simple ester or compounds having multiple ester groupings, such as complex esters, polyesters or diesters. These esters are made from mono- and polyhydroxy alkanols and alkane carboxylic acids, frequently of about 4 to 12 carbon atoms.

The reaction product of a monohydroxy alcohol and a monocarboxylic acid is usually considered to be a simple ester. A diester is usually considered to be the reaction product of 1 mole of a dicarboxylic acid, say of 6 to 10 carbon atoms, with 2 moles of a monohydric alcohol or 1 mole of a glycol of 4 to 10 carbon atoms with two moles of a monocarboxylic acid of 4 to 10 carbon atoms. The diesters frequently contain from 20 to 40 carbon atoms. One complex ester is of the type



in which X represents a monohydric alcohol residue, Y represents a dicarboxylic acid residue and Z represents a glycol residue and the linkages are ester linkages. Those esters, wherein X represents a monoacid residue, Y represents a glycol residue and Z represents a dibasic acid residue are also considered to be complex esters. The complex esters often have 30 to 50 carbon atoms. Polyesters, or "polyester bright stocks" can be prepared by direct esterification of dibasic acids with glycols in about equimolar quantities. The polyesterification reaction is usually continued until the product has a kinematic viscosity from about 15 to 200 centistokes at 210° F., and preferably 40 to 130 centistokes at 210° F.

Although each of these products in itself is useful as a lubricant, they are also useful when added or blended with each other in synthetic lubricant compositions. These esters and blends have been found to be especially adaptable to the conditions to which turbine engines are exposed, since they can be formulated to give a desirable combination of high flash point, low pour point, and high viscosity at elevated temperatures. In addition, many complex esters have shown good stability to shear. There may also be included in the blends up to about 1% or more by weight of a foam inhibitor such as a methyl silicone polymer or other additives to provide a particular characteristic, for instance, extreme pressure or load carrying agents, corrosion inhibitors, etc.

Typical synthetic lubricants may be formulated essentially from a major amount—about 60 to 85%—of a complex ester and a minor amount—about 15 to 40%—of a diester, by stirring together a quantity of diester and complex ester at an elevated temperature, altering the proportions of each component until the desired viscosity is reached. Polyesters can be employed to thicken diester base stocks to increase the load carrying capacity of the base diester oil. The polyester will generally not comprise more than about 50 weight percent of the blend, preferably about 20 to 35 weight percent. Usually the amount of the polyester employed in any blend would be at least about 5%, and the majority of the lubricant is a diester. Other polymers such as Acryloids may be

added as thickeners to the esters, generally the simple esters such as the above diesters, to obtain a base oil of desired viscosity. The Acryloids are polymers of mixed C<sub>4</sub> to C<sub>18</sub> esters of methacrylic acid having 10,000 to 20,000 molecular weight. Advantageously, the final lubricating oil composition would have a maximum viscosity at —40° F. of about 13,000 centistokes and a minimum viscosity of about 3.5 centistokes at 210° F.

The monohydric alcohols employed in these esters usually contain less than about 20 carbon atoms and are generally aliphatic. Preferably, the alcohol contains up to about 12 carbon atoms. Useful aliphatic alcohols include butyl, hexyl, methyl, iso-octyl and dodecyl alcohols, C<sub>13</sub> oxo alcohols and octadecyl alcohols. C<sub>8</sub> to C<sub>10</sub> branched chain primary alcohols are frequently used to improve the low temperature viscosity of the finished lubricant composition. Alcohols such as n-decanol, 2-ethylhexanol, "oxo" alcohols, prepared by the reaction of carbon monoxide and hydrogen upon the olefins obtainable from petroleum products such as diisobutylene and C<sub>7</sub> olefins, ether alcohols such as butyl carbitol, tripropylene glycol mono-isopropyl ether, dipropylene glycol mono-isopropyl ether, and products such as "Tergitol 3A3," which has the formula C<sub>13</sub>H<sub>27</sub>O(CH<sub>2</sub>CH<sub>2</sub>O)<sub>3</sub>H, are suitable alcohols for use to produce the desired lubricant. Iso-octanol and iso-decanol are alcohol mixtures made by the oxo process from C<sub>3</sub> to C<sub>4</sub> copolymer heptenes. The cut which makes up iso-octanol usually contains about 17% 3,4-dimethylhexanol; 29% 3,5-dimethylhexanol; 25% 4,5-dimethylhexanol; 1.4% 5,5-dimethylhexanol; 16% of a mixture of 3-methylheptanol and 5-ethylheptanol; 2.3% 4-ethylhexanol; 4.3%  $\alpha$ -alkyl alkanols and 5% other materials.

Generally, the glycols contain from about 4 to 12 carbon atoms; however, if desired they could contain a greater number. Among the specific glycols which can be employed are 2-ethyl-1,3-hexanediol, 2-propyl-3,3-heptanediol, 2-methyl-1,3-pantanediol, 2-butyl-1,3-butanediol, 2,4-diphenyl-1,3-butanediol, and 2,4-dimesityl-1,3-butanediol. In addition to these glycols, other glycols may be used, for instance, where the alkylene radical contains 2 to 4 carbon atoms such as diethylene glycol, dipropylene glycol and other glycols up to 1,000 to 2,000 molecular weight. The most popular glycols for the manufacture of ester lubricants appear to be polypropylene glycols having a molecular weight of about 100 to 300 and 2-ethyl hexanediol. The 2,2-dimethyl glycols, such as neopentyl glycol have been shown to impart heat stability to the final blends. Minor amounts of other glycols or other materials can be present as long as the desired properties of the product are not unduly deleteriously affected.

Aside from glycols, the esters may be made from polyhydric alcohols of more than two hydroxyl groups, e.g. tri- and tetrahydroxy aliphatic alcohols having about 4 to 12 carbon atoms, preferably about 5 to 8 carbon atoms; for instance, pentaerythritol, trimethylolpropane and the like. Particularly suitable ester base oils are formed when these alcohols are reacted with monocarboxylic acids having about 4 to 12 carbon atoms, preferably 4 to 9 carbon atoms. It is preferred that the reaction be conducted so as to substantially completely esterify the acids.

One group of alcanoic acids includes those of 6 to 24 carbon atoms such as stearic, lauric, etc. The carboxylic acids employed in making ester lubricants will often contain from about 4 to 12 carbon atoms. Suitable acids are described in U.S. Patent No. 2,575,195 and include the aliphatic dibasic acids of branched or straight chain structures which are saturated or unsaturated. The preferred acids are the saturated aliphatic carboxylic acids containing not more than about 12 carbon atoms, the mixtures of these acids. Such acids include succinic, adipic, suberic, azelaic and sebatic acids and "isosebacic" acid which is a mixture of  $\alpha$ -ethyl suberic acids,  $\alpha,\alpha$ -diethyl adipic acid and sebatic acid. This composite of acids is attractive from the viewpoint of economy and

availability since it is made from petroleum hydrocarbons rather than the natural oils and fats which are used in the manufacture of many other dicarboxylic acids, which natural oils and fats are frequently in short supply. The preferred dibasic acids are sebacic and azelaic or mixtures thereof. Minor amounts of adipic used with a major amount of sebacic may also be used with advantage.

Various useful ester base oils are disclosed in U.S. Patents Nos. 2,499,983; 2,499,984; 2,575,195; 2,575,196; 2,703,911; 2,705,724 and 2,723,286. Generally, the synthetic base oils consist essentially of carbon, hydrogen and oxygen, i.e. the essential nuclear chemical structure is formed by these elements alone. However, these oils may be substituted with other elements such as halogens, e.g. chlorine and fluorine. Some representative components of ester lubricants are ethyl palmitate, ethyl stearate, di(2-ethylhexyl) sebacate, ethylene glycol dilaurate, di(2-ethylhexyl) phthalate, di(1,3-methyl butyl) adipate, di(2-ethyl butyl) adipate, di(1-ethyl propyl) adipate, diethyl oxylate, glycerol tri-n-octoate, di-cyclohexyl adipate, di-(undecyl) sebacate, tetra-ethylene glycol-di-(2-ethylene hexoate), di-Cellosolve phthalate, butyl phthalyl butyl glycolate, di-n-hexyl fumarate polymer dibenzyl sebacate, and diethylene glycol bis(2-n-butoxy ethyl carbonate). 2-ethylhexyl-adipate-neopentyl glycidate-2-ethylhexyl is a representative complex ester.

The esters are manufactured, in general, by mere reaction of the alcoholic and acidic constituents, although simple esters may be converted to longer chain components by transesterification. The constituents, in the proportions suitable for giving the desired ester, are reacted preferably in the presence of a catalyst and solvent or water entraining agent to insure maintenance of the liquid state during the reaction. Aromatic hydrocarbons such as xylene or toluene have proven satisfactory as solvents. The choice of solvent influences the choice of temperature at which the esterification is conducted; for instance, when toluene is used a temperature of 140° C. is recommended; with xylene, temperatures up to about 195° C. may be used. To provide a better reaction rate an acid esterification catalyst is often used. Many of these catalysts are known and include, for instance, HCl, H<sub>2</sub>SO<sub>4</sub>, NaHSO<sub>4</sub>, aliphatic and aromatic sulfonic acids, phosphoric acid, hydrobromic acid, HF and dihydroxyfluoboric acid. Other catalysts are thionyl chloride, boron trifluoride and silicon tetrafluoride. Titanium esters also make valuable esterification and transesterification catalysts.

In a preferred reaction about 0.5 to about 1 weight percent, or advantageously, 0.2 to 0.5% of the catalyst is used with xylene solvent at a temperature of 165 to 200° C. while refluxing water. The temperatures of the reaction must be sufficient to remove the water from the esterification mass as it is formed. This temperature is

usually at least about 140° C. but not so high as to decompose the wanted product. The highest temperature needed for the reaction will probably be about 200° C., preferably not over about 175° C. The pressure is conveniently about atmospheric. Although reduced pressure or superatmospheric pressure could be utilized, there is usually no necessity to use reduced pressures, as the temperatures required at atmospheric pressure to remove the water formed do not usually unduly degrade the product.

When reacting glycols with dibasic acids to produce a polyester, it is preferred to continue the reaction with concomitant boiling off of water from the reaction mixture until the polyester product has a kinematic viscosity of about 15 to 200 centistokes at 210° F., preferably about 40 to 130 centistokes. When this point has been reached, the polymerization can be stopped, for instance, by adding a "capping alcohol" to the reaction mixture, and continuing to reflux until water ceases to be evolved. The capping alcohol is a low molecular weight mono-alcohol of up to about 20 carbon atoms. It is standard practice, when esters are made using the conventional acid catalysts such as sodium bisulfate or paratoluene-sulfonic acid, to give the esters an after-treat by washing the ester with a 5% aqueous K<sub>2</sub>CO<sub>3</sub> solution or by heating the ester in an autoclave for 15 hours at 340 to 350° F. with 10 weight percent of propylene oxide. It is also conventional to subject the ester to filtration to remove insoluble materials. After this the product may be subjected to a reduced pressure distillation or stripping at 100° to 200° C. to remove volatile materials, such as water, the solvent and light ends.

The following examples are included to further illustrate the present invention.

Samples of an ester based fluid containing phenyl- $\alpha$ -naphthylamine (abbreviated PAN) or an N-substituted compound identified in Table I below and samples containing both of the additives were subjected to oxygen absorption tests at 450° F. The ester fluid was composed of a blend of 80% complex ester prepared from 1 mole neopentyl glycol, 2 moles of azelaic acid and 2 moles iso-octyl alcohol and 20% diiso-octyl azelate.

The oxygen absorption tests were conducted by passing a stream of oxygen at the rate of 1 cubic foot per hour through 75 grams of the samples and noting the total time (T<sub>t</sub>) in minutes required to absorb 2500 milliliters of oxygen and the induction period (T<sub>i</sub>) in minutes. The induction time is the period during which often a minor portion of the oxygen is absorbed by the fluid and its end is signalled by a marked increase in the rate of oxygen absorption. Also noted is the volume of O<sub>2</sub> absorbed during the induction period and is identified in the table as V<sub>i</sub>.

The results of these tests are shown in Table I.

TABLE I

| Sample No. | Additives                                   | Wt. percent | T <sub>i</sub> | T <sub>t</sub> | V <sub>i</sub> |
|------------|---------------------------------------------|-------------|----------------|----------------|----------------|
| 1-----     | PAN                                         | 0.5         | 75.6           | 163            | 217            |
| 2-----     | 2-aminopyridine                             | 0.5         | 90.6           | 148            | 602            |
| 3-----     | PAN                                         | 0.5         |                |                |                |
| 4-----     | 3-aminoquinoline                            | 1.0         | 75.0           | 130            | 500            |
| 5-----     | PAN                                         | 0.5         |                |                |                |
| 6-----     | Benzylidene 2,2'-di-(4-picoly)amine         | 1.0         |                | 304            | 705            |
| 7-----     | PAN                                         | 0.5         | 248            |                |                |
| 8-----     | Benzylidene 2,2'-di-(4-picoly)amine         | 0.2         |                | 218            | 730            |
| 9-----     | PAN                                         | 0.5         | 168            |                |                |
| 10-----    | Benzylidene 2,2'-di-(4-picoly)amine         | 0.2         |                | 81             | 0              |
| 11-----    | 2-anilinopyridine                           | 1.0         | 12             | 234            | 1,060          |
| 12-----    | PAN                                         | 0.5         | 186            |                |                |
| 13-----    | 2-(N-tertbutylamino)-4-picoline             | 1.0         |                | 271            | 782            |
| 14-----    | PAN                                         | 0.5         | 210            |                |                |
| 15-----    | 2-anilinoquinoline                          | 1.0         |                | 210            | 1,150          |
| 16-----    | PAN                                         | 0.5         | 165            |                |                |
| 17-----    | 2-anilinoquinoline                          | 1.0         |                | 109            | 0              |
| 18-----    | 2,6-di(2-pyridylaminomethyl)4-t-octylphenol | 1.0         | 14             | 281            | 884            |
| 19-----    | PAN                                         | 0.5         | 211            |                |                |
| 20-----    | 2,6-di(2-pyridylaminomethyl)4-t-octylphenol | 0.2         |                | 176            | 640            |
| 21-----    | PAN                                         | 0.5         | 122            |                |                |

The data of Table I show that phenylnaphthylamine and the N-substituted amino compounds of the present invention when used alone are relatively ineffective antioxidants. However, when the two additives are used in combination it is seen from the data that the ester based fluid is endowed with unusual antioxidant characteristics.

Two synthetic lubricant formulations identified in Table II below were subjected to the MIL-L-7808 oxidation corrosion test. The ester base fluid of the formulations was the same fluid blend employed in the oxygen absorption test above.

The results of the tests are shown below:

TABLE II.—OXIDATION-CORROSION TEST DATA  
(347° F., 72 HRS.)

| Sample No.                         | 5      | 12     |
|------------------------------------|--------|--------|
| Additives, percent:                |        |        |
| (1)                                | 1.05   | 1.05   |
| (2)                                | 2.02   | 3.02   |
| New oil:                           |        |        |
| KV/100 cs.                         | 36.37  | 36.31  |
| Acid No.                           | 0.13   | 0.15   |
| Used oil:                          |        |        |
| KV/100 cs.                         | 38.22  | 37.76  |
| Acid No.                           | 0.90   | 0.43   |
| Changes:                           |        |        |
| KV/100, percent                    | 5.23   | 4.00   |
| Acid No.                           | 0.77   | 0.28   |
| Wt. change, mg./cm. <sup>2</sup> : |        |        |
| Al alloy                           | +0.038 | +0.007 |
| Mg alloy                           | -0.046 | -0.015 |
| Steel                              | +0.046 | 0.0    |
| Copper                             | -0.031 | -0.015 |
| Silver                             | +0.031 | +0.007 |

<sup>1</sup> PAN.

<sup>2</sup> Benzylidene 2,2'-di-(4-picoly)amine.

<sup>3</sup> 2,6-di(2-pyridyl-amino-methyl)4-t-octylphenol.

The data of Table II show that the compositions of the present invention exhibit acceptable metal corrosion characteristics and small increases in viscosity and acid number as well.

It is claimed:

1. A lubricating oil composition consisting essentially of an ester based synthetic fluid of lubricating viscosity, about 0.01 to 5% by weight of an ester based fluid-soluble aromatic amine having the general formula:



wherein Q is a monovalent aromatic hydrocarbon radical of 6 to 20 carbon atoms and Q' is an aromatic hydrocarbon radical of 6 to 16 carbon atoms and about 0.01 to 5% by weight of an N-substituted amino-compound represented by the general formula:



wherein X is selected from the group consisting of pyridyl and quinolyl radicals; R is an n-valent aromatic hydrocarbon radical of 6 to 24 carbon atoms, and n is 1 to 2, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

2. The composition of claim 1 wherein the aromatic amine is phenylnaphthylamine.

3. A lubricating oil composition consisting essentially of an ester based synthetic fluid of lubricating viscosity, about 0.01 to 5% by weight of an ester based fluid-soluble aromatic amine having the general formula:



wherein Q is a monovalent aromatic hydrocarbon radical of 6 to 20 carbon atoms and Q' is an aromatic hydrocarbon radical of 6 to 16 carbon atoms and about 0.01 to

5

5% by weight of an ester based fluid-soluble N-substituted aminopyridine having the structural formula:



wherein R<sub>1</sub> is selected from the group consisting of hydrogen and lower alkyl and R<sub>2</sub> is an aryl group of 6 to 12 carbon atoms, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

4. A lubricating oil composition consisting essentially of an ester based synthetic fluid of lubricating viscosity, about 0.01 to 5% by weight of an ester based fluid-soluble aromatic amine having the general formula:



wherein Q is a monovalent aromatic hydrocarbon radical of 6 to 20 carbon atoms and Q' is an aromatic hydrocarbon radical of 6 to 16 carbon atoms and about 0.01 to 5% by weight of an ester based fluid-soluble N-substituted aminoquinoline compound having the structural formula:



wherein R<sub>1</sub> is hydrogen and R<sub>2</sub> is an aryl group of 6 to 12 carbon atoms and R<sub>1</sub> and NHR<sub>2</sub> are on different carbon atoms of the positions 2 to 8, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

5. A lubricating oil composition consisting essentially of an ester based synthetic fluid of lubricating viscosity, about 0.01 to 5% by weight of an ester based fluid-soluble aromatic amine having the general formula:



wherein Q is a non-olefinic, non-acetylenic monovalent hydrocarbon of 1 to 20 carbon atoms and Q' is an aromatic hydrocarbon radical of 6 to 16 carbon atoms and about 0.01 to 5% by weight of an ester based fluid-soluble aromatic amine having the general formula:



wherein R<sub>1</sub> is an alkyl group of 1 to 12 carbon atoms and R<sub>3</sub> is an aryl group of 6 to 12 carbon atoms, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

6. A lubricating oil composition consisting essentially of an ester based synthetic fluid of lubricating viscosity, about 0.01 to 5% by weight of an ester based fluid-soluble aromatic amine having the general formula:



wherein Q is a non-olefinic, non-acetylenic monovalent hydrocarbon of 1 to 20 carbon atoms and Q' is an aromatic hydrocarbon radical of 6 to 16 carbon atoms and about 0.01 to

75

5

5

60

65

70

75

about 0.01 to 5% by weight of an ester based fluid-soluble aromatic amine having the general formula:



wherein R<sub>1</sub> is hydrogen; R<sub>4</sub> is a divalent alkyl radical of 1 to 4 carbon atoms and R<sub>5</sub> is an alkyl group of 1 to 8 carbon atoms, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

7. A lubricating oil composition consisting essentially of an ester based synthetic fluid of lubricating viscosity, about 0.01 to 5% by weight of phenylnaphthylamine and about 0.01 to 5% by weight of 2-anilinoquinoline, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

8. A lubricating oil composition consisting essentially of an ester based synthetic fluid of lubricating viscosity, about 0.01 to 5% by weight of phenylnaphthylamine and about 0.01 to 5% by weight of 2-anilinopyridine, said amounts being sufficient to retard oxidation of said ester base fluid at 450° F. and said ester base fluid being an ester of an alkanol of 4 to 12 carbon atoms and an alkane carboxylic acid of 4 to 12 carbon atoms.

9. A lubricating oil composition consisting essentially of an ester based synthetic fluid of lubricating viscosity, about 0.01 to 5% by weight of phenylnaphthylamine and about 0.01 to 5% by weight of 2-(N-benzylamino)4-picoline, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

10. A lubricating oil composition consisting essentially of an ester based synthetic fluid of lubricating viscosity, about 0.01 to 5% by weight of phenylnaphthylamine and about 0.01 to 5% by weight of benzylidene-2,2'-di(4-picolyl)amine, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

11. A lubricating oil composition consisting essentially of an ester based synthetic fluid of lubricating viscosity, about 0.01 to 5% by weight of phenylnaphthylamine and about 0.01 to 5% by weight of 2,6-di(2-pyridylamino-methyl)4-tertiary octyl phenol, said amounts being sufficient to retard oxidation of said ester based fluid at 450° F. and said ester based fluid being an ester of an alkanol of 4 to 12 carbon atoms and an alkane carboxylic acid of 4 to 12 carbon atoms.

20

#### References Cited by the Examiner

##### UNITED STATES PATENTS

|           |         |                |            |
|-----------|---------|----------------|------------|
| 2,136,788 | 11/1938 | Fairlie        | 252—50     |
| 2,198,961 | 4/1940  | Dietrich       | 252—50 X   |
| 2,290,032 | 7/1942  | Burk           | 252—50 X   |
| 2,318,196 | 5/1943  | Chenicek       | 44—63      |
| 2,336,006 | 12/1943 | Fuller         | 252—51.5   |
| 2,361,339 | 10/1944 | White et al.   | 252—51.5   |
| 2,363,778 | 11/1944 | Pedersen       | 44—63      |
| 2,459,112 | 1/1949  | Oberright      | 252—51.5   |
| 2,637,636 | 5/1953  | Walters        | 44—63      |
| 2,933,379 | 4/1960  | Fields         | 44—63      |
| 3,043,783 | 7/1962  | Hatcher et al. | 252—51.5 X |
| 3,093,585 | 6/1963  | Low et al.     | 252—51.5 X |
| 3,121,691 | 2/1964  | Eickemeyer     | 252—51.5   |

DANIEL E. WYMAN, *Primary Examiner.*

P. P. GARVIN, *Assistant Examiner.*